

March 21, 1961

G. T. ANGELOFF

2,976,195

SUPER PRESSURE ELECTRODE-INSULATOR

Filed Jan. 20, 1958



FIG - 2



FIG - 1



FIG - 3

INVENTOR.

GEORGE T. ANGELOFF

BY

*Ronald S. Shubler*

# United States Patent Office

2,976,195

Patented Mar. 21, 1961

1

2,976,195

## SUPER PRESSURE ELECTRODE-INSULATOR

George T. Angeloff, North Branford, Conn., assignor to Olin Mathieson Chemical Corporation, a corporation of Virginia

Filed Jan. 20, 1958, Ser. No. 709,954

5 Claims. (Cl. 148—135)

The present invention relates to electrodes and in particular to the manufacture of electrode-insulator assemblies capable of withstanding super pressures; i.e., pressures of the order of 50,000 lbs. per square inch.

A particular feature of the invention is the provision of a novel method of manufacturing such an electrode-insulator assembly.

Another feature of the invention is the provision of a process for the manufacture of an electrode-insulator assembly which includes the step of firing the insulator and hardening the metal housing surrounding the insulator in one operation.

A still further feature of the invention is the provision of a process useful in the manufacture of electrode-insulator assemblies which is effective, when the insulator is disposed within a housing, to seat the entire exterior surface or face of the insulator against a corresponding surface of the housing without the need for grinding and lapping.

Another feature of the invention is the provision of a process in the manufacture of electrode-insulators which is inexpensive to practice.

A process embracing the principles of the present invention may comprise the steps of providing a heat hardenable metallic housing having a tapered bore, providing an unfired ceramic insulator, machining a taper on the outer surface of the insulator corresponding to the taper of said tapered bore, inserting the unfired insulator into the metallic housing so that the tapers mate, and heating the assembled insulator and housing to fire the insulator and to harden the housing.

Other features and advantages of the present invention will become more apparent from a study of the succeeding specification when read in conjunction with the appended drawings, in which:

Fig. 1 is a mid-sectional view of an electrode-insulator assembly manufactured in accordance with the process of the present invention;

Fig. 2 is a mid-sectional view of an insulator and its housing illustrating the disposition of the elements at the time of firing;

Fig. 3 is a mid-sectional view of the insulator, and;

Fig. 4 is a side view of the electrode.

Referring now to Fig. 1 there is shown a typical super pressure electrode-insulator assembly including a housing 10, an insulator 11, and an electrode 12, an insulating washer 13, a lock nut 14, and a terminal nut 16.

It is to be understood that although the material from which the insulator in the exemplary embodiment of the invention is made is known as Lava-Grade A, supplied by the American Lava Corporation, Chattanooga, Tennessee, a variety of other ceramics may be substituted.

Examples of such other ceramics are steatite, cordierite, mullite and the like.

Correspondingly, although the present embodiment of the invention calls for a steel housing fabricated from 440 "C" stainless, it is entirely within the scope of the invention to substitute any heat hardenable steel.

2

In the practice of the present invention the steel housing 10 is provided with a tapered bore 17 where the included angle subtended by the taper falls within the minimum value of 5° and the maximum value of 90°.

5 In the illustrated embodiment of the invention the included angle is about 10°.

A length of unfired Grade A Lava is machined to the general configuration shown in Fig. 3. A taper having a 10° included angle is formed on the exterior surface and the interior is bored and counterbored to provide a sliding fit for the electrode 12 of Fig. 4.

Next the unfired insulator is placed within the housing 10 as shown in Fig. 2 and thereafter the assembly is disposed within a cool furnace so that the larger diameter of the insulator is facing upwardly. Preferably, but not necessarily, a light weight W, in this instance a 20 gram weight, is disposed as shown in Fig. 2 to urge the insulator into contact with the housing.

An atmosphere of nitrogen is then introduced to the furnace. As is well known in the art nitrogen is utilized to prevent oxidation and to provide a generally inert atmosphere. Thereafter the furnace temperature is raised to about 1950° F. at a rate not exceeding 500° per hour. The 1950° temperature is held for about 30 minutes. Next the source of heat is cut off and the assembly is oven cooled to about 250° F. before removal from the furnace.

Upon removal from the furnace, an examination of the stainless steel housing reveals a hardness of 42 to 30 44 Rockwell C Scale while the electrical resistance of the assembly measured from the electrode 12 to the housing 10 is of the order of 15 megohms.

A static pressure of about 50,000 pounds per square inch applied to the insulator-electrode assembly, as shown 35 in Fig. 1, and in a direction which tends to urge the insulator towards the small diameter of the taper is effective to move the insulator into snug contact with its housing (usually approximately 0.010 inch measured along the longitudinal axis of the assembly) does not 40 fail the insulator.

Correspondingly, when the unit is placed in threaded engagement with a high pressure vessel and used in the fashion of a spark plug to ignite a monopropellant charge, the ceramic insulator stands up well. Dynamic pressures in excess of 50,000 pounds per square inch have 45 no harmful effect upon the electrode-insulator assembly.

It is to be understood that the process of the present invention may be utilized to insulate or to develop electrode-insulator assemblies useful in other fields such 50 as, for example, the provision of a super pressure plug for housing a thermocouple where the thermocouple is insulated from its housing in the same fashion that the electrode 12 is so insulated.

It is especially important to note that the practice of the present process steps provide an inexpensive way to 55 provide an insulated electrode which is operable in super pressure ranges. Heretofore, it has been necessary to laboriously grind and lap fired ceramic insulators with respect to a metallic housing so as to provide uniform 60 surface contact between the insulator and its housing to avoid stress concentrations which crack the insulator.

It is anticipated that a variety of electrode-insulator assemblies may be devised with the practice of the process steps of the present invention without departing from 65 the spirit and scope thereof.

What is claimed is:

1. A process for manufacturing a super pressure insulated electrode capable of withstanding shock pressures of the order of 50,000 p.s.i. generated over intervals as short as  $\frac{1}{2}$  millisecond comprising the steps 70 of providing a heat hardenable metallic housing having a tapered bore, said housing being fabricated of type

440 stainless steel, providing an unfired ceramic insulator, machining a taper on the outer surface of the insulator corresponding to the tapered bore of the housing, inserting the unfired insulator into the metallic housing so that the taper and the tapered bore mate, and heating the assembled insulator and housing to a temperature of about 1950° F. at a rate not exceeding 500° per hour to fire the insulator and to harden the housing and furnace cooling the insulated electrode to about 250° F.

2. A process for manufacturing a super pressure insulated electrode capable of withstanding shock pressures of the order of 50,000 p.s.i. generated over intervals as short as  $\frac{1}{2}$  millisecond comprising the steps of providing a heat hardenable metallic housing having a tapered bore, said housing being fabricated of type 440 stainless steel, providing an unfired ceramic insulator, machining a taper on the outer surface of the insulator corresponding to the tapered bore of the housing, inserting the unfired insulator into the metallic housing so that the taper and the tapered bore mate, applying pressure upon the ceramic insulator which tends to move the insulator relative to the housing and heating the assembled insulator and housing to a temperature of about 1950° F. at a rate not exceeding 500° per hour to fire the insulator and to harden the housing and furnace cooling the insulated electrode to about 250° F.

3. A process for manufacturing a super pressure insulated electrode capable of withstanding shock pressures of the order of 50,000 p.s.i. generated over intervals as short as  $\frac{1}{2}$  millisecond comprising the steps of providing a heat hardenable metallic housing having a tapered bore, said housing being fabricated of type 440 stainless steel, providing an unfired ceramic insulator, machining a taper on the outer surface of the insulator corresponding to the tapered bore of the housing, inserting the unfired insulator into the metallic housing so that the taper and the tapered bore mate, applying pressure upon the ceramic insulator which tends to move the insulator relative to the housing and applying heat to the assembled insulator and housing to a temperature of about 1950° F. at a rate of about 500° per hour to fire the insulator and to harden the housing and furnace cooling the insulated electrode to about 250° F.

4. A process for manufacturing a super pressure in-

sulated electrode capable of withstanding shock pressures of the order of 50,000 p.s.i. generated over intervals as short as  $\frac{1}{2}$  millisecond comprising the steps of providing a heat hardenable stainless steel housing having a tapered bore, said housing being fabricated of type 440 stainless steel, providing an unfired ceramic insulator, machining a taper on the outer surface of the insulator corresponding to the tapered bore of the housing, inserting the unfired insulator into the metallic housing so that the taper and the tapered bore mate, disposing the assembled insulator and housing so that the taper flares upwardly and outwardly, applying pressure upon the ceramic insulator which tends to move the insulator relative to the housing and heating the assembled insulator and housing to a temperature of about 1950° F. at a rate not exceeding 500° per hour in a nitrogen atmosphere to fire the insulator and to harden the housing and furnace cooling the insulated electrode to about 250° F.

5. A process for manufacturing a super pressure insulated electrode capable of withstanding shock pressures of the order of 50,000 p.s.i. generated over intervals as short as  $\frac{1}{2}$  millisecond comprising the steps of providing a heat hardenable metallic housing having a tapered bore, said housing being fabricated of type 440 stainless steel, providing an unfired ceramic insulator, machining a taper on the outer surface of the insulator corresponding to the tapered bore of the housing, inserting the unfired insulator into the metallic housing so that the taper and the tapered bore mate, and heating the assembled insulator and housing to a temperature of about 1950° F. at a rate not exceeding 500° per hour in an atmosphere of nitrogen to fire the insulator and to harden the housing and furnace cooling the insulated electrode to about 250° F.

35

#### References Cited in the file of this patent

#### UNITED STATES PATENTS

|           |                       |               |
|-----------|-----------------------|---------------|
| 974,008   | Wolff                 | Oct. 25, 1910 |
| 2,469,211 | Schwartzwalder et al. | May 3, 1949   |
| 2,699,158 | Purdy et al.          | Jan. 11, 1955 |
| 2,784,112 | Nicholson             | Mar. 5, 1957  |

#### OTHER REFERENCES

Republic Enduro Stainless Steels, Republic Steel Corp.,  
45 pages 48-52, 1951.